

Feb. 2, 1965

F. W. BRODERICK

3,167,850

TRANSFER ROLL

Filed Dec. 21, 1962

FIG. 1



FIG. 2



FIG. 3



FIG. 4



1

3,167,850

**TRANSFER ROLL**

Frank W. Broderick, P.O. Box 2, Stirling, N.J.  
Filed Dec. 21, 1962, Ser. No. 246,627  
3 Claims. (Cl. 29—121)

This invention relates to an engraved metal roll having patterned cavities therein adapted to uniformly transfer metered amounts of solution to a non-woven fabric in tangential contact therewith.

In the manufacture of non-woven fabric from long filaments of rayon and other artificial fibers it is necessary to adhere the parallel disposed fibers to one another by means of a uniformly applied adhesive.

The method presently employed is to transfer the solution to the continuously moving web by means of an engraved steel roll, rotating in a fountain and disposed in conjunction with a back up roll, generally rubber covered. The non-woven fabric passes between the nip of line contact between said rolls and in doing so picks up by absorption a uniform amount of solution.

The engraved design disposed on the application roll is of such depth and configuration as to transfer the solution to the non-woven fabric, in extremely closely held tolerances, said solution being then spread by capillary action in given areas to yield a moistened binding channel having a uniform amount of solution per square inch.

The production of non-woven fabric is big business, as the material is used for disposable diapers, sanitary napkins, suit paddings, wiper cloths, napkins, etc.

The present method of making engraved transfer rolls is by means of a conventional mill and die wherein a small female roll is first prepared and from this a co-acting small male roll is made. This male roll of a few inches in length is then repeatedly linearly transferred to the surface of a large, sometimes six to ten feet long, production roll. Clearly, this procedure is very expensive since it requires highly skilled labor and is very cumbersome and time consuming.

Attempts have been made to produce a suitable acid etched engraved transfer roll using conventional acid resist coatings but the resulting embossed cavities of the pattern were provided with undesirable saw tooth or ragged edges which engaged or picked up the tiny filaments of the fabric, a highly undesirable result.

Accordingly, it is impossible to produce satisfactory acid etched embossed steel transfer rolls of the type desired above before this invention was made.

In the conventional method of etching steel rolls, as described for example in Broderick U.S. 2,887,042, a relatively soft steel roll is photo-engraved and then acid etched to the desired depth and finally heat hardened to withstand usage.

This invention reverses the prior art and in so doing produces a new process with unobvious desirable results.

According to this invention the soft steel roll is suitably heat hardened before it is photo-engraved. This heat hardening, it was found, refined the steel grain structure so that the roll could be now acid etched to produce smooth cavities having straight and uniform edges in lieu of the prior art saw tooth edges and irregular depths.

It is an object of this invention to produce acid etched engraved metal transfer rolls for the transfer of uniform amounts of solution to non-woven fabric, the cavities thereof having smooth, straight or snag proof edges.

It is another object to provide an inexpensive snag proof transfer roll.

It is a further object to provide an engraved pattern having great accuracy and uniform depth of cavities.

These and other objectives of this invention will become apparent upon reading the following descriptive disclosure taken in conjunction with the accompanying drawing in which:

2

FIG. 1 is a diagrammatic perspective view of a schematic engraved roll disposed in part in a fountain containing the binder or adhesive solution and showing the use of a doctor blade to scrape off excess solution from the surface,

FIG. 2 is a cross-section view of a heat hardened acid etched metal roll showing the smooth, accurate edges and smooth, rounded internal contour of a single linear cavity as produced by this invention,

FIG. 3 is a section view of the roll of FIG. 2 after being chrome plated, showing the manner of chrome plating building up on the round edges of the cavities, and

FIG. 4 is the cross-section view of the roll of FIG. 3 after the built-up or hump-like rounded edges have been polished off to produce a chrome plated transfer roll of uniform radius.

In the use of this invention there is employed a binder or adhesive solution used to bind or adhere the non-woven fibers together. This solution is disposed in a trough or fountain and the embossed transfer roll is partly placed therein. A doctor blade engages the smooth surface of the transfer roll and removes the excess solution thereon. The amount of solution transferred to the web is critical since too little solution will not effect a binding together of the fibrous filaments and too much solution produces a stiff undesirable non-woven fabric.

Turning now to the drawing, a conventional fountain 10 is provided with a conventional doctor blade 11 secured removably thereto. An embossed transfer roll 12, for example of herringbone pattern, is disposed partly in the fountain 10. A continuously moving web 13 of non-woven fibers is passed tangentially over the top of the embossed transfer roll 12 and engages on its opposed side a backup roll 14. The binder solution strikes through the non-woven fabric to the opposite side thereof binding the long fibers in the manner similar to that of a stitched line. In short, the binder solution from the rotating cavities is transferred to the moving web and in effect stitches the long fibers laterally to form a semi-quilted soft non-woven fabric.

To effect this critical uniformity of binder, the engraved rolls must have a precisely predetermined pattern and this pattern must accurately transfer a critical amount of solution per lateral area or circumferential surface.

According to this invention, a polished suitable high carbon steel or steel alloy roll is heat hardened, preferably by flame hardening to a desired fine grain structure. Preferably this desired fine grain structure is produced throughout the steel roll. However, a fine grain structure in the surface of suitable depth on the radius is operable.

This fine grain structure is homogeneous throughout the pattern area and depth and is essential and critical to the success of this invention.

By way of an illustrative embodiment of this invention a smooth surfaced forged chrome-molybdenum steel roll, AISI 4150, having the following composition:

Carbon range 0.45—0.55% by weight  
Manganese range 0.60—0.90% by weight  
Phosphorous (maximum) 0.040% by weight

60 Sulfur (maximum) 0.050% by weight  
Chromium range, about 0.80 to about 1.10% by weight  
Molybdenum range, about 0.15 to about 0.25% by weight

was flame hardened to a critical transformation temperature of 1575° F. to produce the desired homogeneous fine grain structure as shown by microscopic examination and by a Rockwell hardness tester C scale reading of 53. At this temperature the finest grain structure was obtained which structure gave the smoothest cavities on acid etching.

Other chrome-molybdenum alloy steels in the range of the AISI 4150 composition are operable. In general, the

alloy steel is heated to within ten (10) degrees Fahrenheit of their final transformation point in order to obtain the desired fine grain structure. Such heat treated steels exhibit a Rockwell C scale hardness reading generally from 45-60 and are operable in this invention. However, in the case of the chrome-molybdenum steels a heat treated alloy treated as above stated preferably has a Rockwell C scale reading of 50 to 55.

In all cases after the alloy is heated to its final transformation temperature it is quenched immediately at this temperature to obtain and retain the desired fine grain structure plus the desired hardness.

Next this smooth surfaced roll was photo-engraved with a desired pattern by means of the conventional lay down process using conventional photo-composing and etching procedures to produce cavities 15 having straight and true edges and smooth, rounded cavities (FIG. 2). These cavities were of uniform smooth depth and of an accuracy of width not obtainable with conventional soft non-heat-treated steel rolls. Moreover, the disastrous saw tooth edges obtained on the soft steel rolls by the prior art were eliminated.

The rollers are then chrome plated to a depth of .0006 to .002 or more inch to produce a chrome plated surface (FIG. 3).

Plating of this thickness and quality tends to build up at the edges of the embossed cavities producing a hump 16 thereon. This hump of chrome is thicker than on the surface and it may be polished off to produce a non-hump slightly rounded edge 17 of uniform chrome plate depth (FIG. 4).

The resultant chrome plated roll is therefore one of uniform depth of cavities, said cavities having round snag-proof edges, said roll having a smooth surface adapted to engage the doctor blade along its entire length.

The transfer rolls prepared according to this invention are operable without being chrome plated. However, the chrome plating of the rolls produces better looking and longer lasting rolls.

This invention has been described by means of several embodiments thereof but is not limited to these illustrations since it is of a generic scope.

I claim:

1. A snag-proof transfer roll of chrome-molybdenum alloy steel engraved for uniform transfer of fluid to a moving monofilament web, said roll having a Rockwell C scale hardness of from 45 to 60 and having a fine grained pre-engraved surface structure obtained by heat treatment to from transformation point to 25° F. above the final transformation temperature of said alloy followed by quenching at said temperature, said chrome molybdenum alloy having a composition of carbon range 0.45 to 0.55 percent by weight, manganese range 0.60 to 0.90 percent by weight, maximum amount of phosphorous 0.40 percent by weight, maximum amount of sulfur 0.050 percent by weight, chromium range about 0.80 to about 1.10 percent by weight and the molybdenum range about 0.15 to about 0.25 percent by weight.

2. The transfer roll of claim 1 wherein the critical transformation temperature is 1575° F. and the Rockwell C scale reading is 53.

3. The transfer roll of claim 1 comprising a smooth surface uniformly deep chrome plating of a depth of .0006 to .002 inch.

#### References Cited by the Examiner

##### UNITED STATES PATENTS

- |           |       |            |
|-----------|-------|------------|
| 2,114,072 | 4/38  | Cleveland. |
| 2,725,640 | 12/52 | Voightman. |
| 2,816,025 | 12/57 | Dahlberg.  |
| 3,048,512 | 8/62  | Nelson.    |

35 WALTER A. SCHEEL, Primary Examiner.

J. D. BEIN, Examiner.